

Patented Apr. 29, 1952

2,594,384

# UNITED STATES PATENT OFFICE

2,594,384

## FUNGI AND BACTERIA RESISTANT PAPER-MAKERS' FELTS AND PROCESS FOR PREPARING SAME

Paul George Benignus, Belleville, Ill., assignor to Monsanto Chemical Company, St. Louis, Mo., a corporation of Delaware

No Drawing. Application November 12, 1946,  
Serial No. 709,105

10 Claims. (Cl. 117—138.5)

1

This invention relates to a process for the treatment of fibrous materials and more specifically to an improved process and composition whereby fibrous materials such as cotton, linen and other cellulosic textiles and fibers, and laid cellulosic materials, and fibrous proteinaceous materials such as woolen textiles and felts, particularly papermakers' felts, may be made highly and permanently resistant to attack by fungi and bacteria.

Papermakers' felts are subject to rapid deterioration due to the activity of fungi and bacteria encountered in the paper mills' white water system, in fact, severe mildew conditions have been experienced whereby the average life of untreated felts has been but one to two weeks, and therefore, a number of preservative treatments have been developed for the purpose of rendering the felts resistant to the deleterious activity of fungi and bacteria. However, in use, these felts are subjected to great volumes of running water and, therefore, the preservatives are continuously and rapidly leached from the felts. There has not been developed, prior to this invention, any preserving treatment for papermakers' felts which will render the felt satisfactorily resistant to the severe leaching action of the paper mills' white water.

When fibrous materials are immersed in a bath containing a fungicidal or a bactericidal agent such as a solution of 8-hydroxyquinoline or a chlorophenol, the treated fibrous material will possess fungicidal and bactericidal properties. However, subsequent wetting, soaking or laundering of the fibrous materials so treated tends to remove the fungicidal or bactericidal agent and thereby substantially reduce the resistance of the fibrous material to the activity of fungi and bacteria. In order to fix the fungicidal agent onto the fabric, it has been proposed to form a difficultly soluble metallic salt of the fungicidal agent within the interstices of the fabric material. Since the metallic salts of many of the fungicidal agents as 8-hydroxyquinoline and the chlorophenols are relatively insoluble in most media for treating fibrous materials, it has been proposed to employ a method whereby after immersion in a water soluble fungicidal agent, some of the metallic salts of which are relatively insoluble, the fabric is drained and subsequently passed through a solution of a water soluble metal salt as calcium, magnesium, or other alkaline earth acetates, zinc, aluminum, copper, cadmium or other heavy metal acetates or nitrates whereby the metal salt of the fungicidal agent is precipitated on or within the fibrous material. This method of fixing the fungicidal agent on the fabric has certain disadvantages. For example, a fabric treated by the two-bath method as has been hereinbefore described and

2

subsequently dried contains soluble salts which leach out when the fibrous material is subsequently laundered or subjected to weathering conditions, and the relatively insoluble salts are 5 not satisfactorily bonded to the fiber, thus the residual protection against fungi and bacteria is materially reduced. On the other hand, many of the best known fungicidal agents such as the heavy metal salts of substances such as oxyquinoline (8-hydroxyquinoline) are too insoluble in 10 water and in other liquid media to be suitable for the impregnation of fibrous materials for the reason that an adequate concentration of the agent cannot be provided in the bath for the 15 proper treatment of the fabric. Also, the use of these heavy metal salts has been impeded for the reason that there has been no satisfactory method for uniformly dispersing and bonding an insoluble fungicide throughout the fibrous material.

One of the objects of the present invention is to provide a novel process whereby fibrous materials such as textiles and more particularly papermakers' felt may be impregnated with sufficient amounts of uniformly dispersed relatively insoluble metallic salts of 8-hydroxyquinoline and derivatives of 8-hydroxyquinoline to render the fibrous material permanently and effectively 20 resistant to the action of fungi and bacteria.

30 A further object is to provide a papermakers' felt treated with a fungicidal composition which felt is highly and permanently resistant to the severe leaching action of continuously running water, particularly, paper mill white water.

35 Other objects will become apparent from the following description and examples:

The improved fungi-proofing process of this invention comprises the preparation of a treating solution by first preparing a water dispersible 40 paste concentrate of a copper, zinc or cadmium salt of an 8-hydroxyquinoline, with a film forming protective colloid such as methyl cellulose in the presence of a wetting agent such as dodecyl benzene sodium sulfonate and dispersing a proper 45 amount of the paste concentrate in a water solution of a water soluble amine-aldehyde resin-forming composition such as an alkyl ether of an alkylol melamine containing an acidic condensation catalyst. Papermakers' felt is then impregnated with the treating solution, for example, by immersing the felt in the solution at room temperature. The felt is subsequently dried and cured for a short time at an elevated temperature. The result of this process up to this point 50 is a uniform deposition of the fungicidal agent on and possibly within the fiber and firmly bonded to the fiber or sealed within the fiber by the film of protective colloid and made water resistant by the melamine or urea-formaldehyde type 55 resin. However, due to the severe leaching action 60

of the large volumes of water encountered in using papermakers' felts, and the abrasive action of the pulp on the felt, I have found that it is necessary to further protect the impregnated felt or fibrous material by giving the felt a further water repelling treatment comprising treating the impregnated felt with an aqueous dispersion comprising a water repelling agent such as an N-methylol alkylamide or an N,N' diacyl diamino methane wherein the alkyl or acyl substituent is a long carbon chain of from C<sub>12</sub> to C<sub>28</sub>, a dispersing agent such as ammonium oleate, triethanol amine oleate, 2-amino-2-methyl-1-propanol oleate or stearate and a water soluble resin-forming composition such as an alkyl ether of mono, di or tetra methylol melamine, for example, the dibutyl ether of tetra methylol melamine or an amine-aldehyde resin-forming composition such as urea-formaldehyde and an acidic catalyst to effect the proper condensation of the resin-forming composition. The treated felt or fibrous material is then dried at 215° F. and heat cured at a temperature of from 250° to 320° F. for 3 to 20 minutes. A papermakers' felt treated in this manner is made highly and permanently resistant to the activity of fungi and bacteria even under the most severe leaching conditions.

The fungicidal agents I have found most desirable for the purpose of this invention are the copper, zinc or cadmium salts of 8-hydroxyquinaline, 5,7-dichlor-8-hydroxyquinaline, or 5,7-dibrom-8-hydroxyquinaline, although other metallic salts may be employed such as the aluminum or calcium salts. However, the copper salts are much to be preferred since they are far more effective from the standpoint of insolubility and permanency when incorporated in the fibrous material. I have found it highly desirable to use these metallic quinolinolates in a very finely divided form of ultimate particle size of from 1 to 10 microns.

While there are many wetting agents which are suitable for the purpose of this invention, I have found the following to be particularly satisfactory: dodecyl benzene sodium sulfonate, decyl benzene succinate, sodium lauryl sulfate, cocoanut oil monoglyceride monosulphate, mixed petroleum sulfonates, and the polyglycol ethers of diisobutylene phenol.

The protective colloid may be selected from methyl cellulose, carboxy methyl cellulose, polyvinyl alcohol, alginates, gelatin, casein, soya proteins, starches, lecithin and water soluble gums. There are, however, many other suitable protective colloids. In general, the methyl cellulose and the carboxy methyl cellulose are most desirable as the protective colloid, not only because they have the desired film-forming properties but they are less susceptible than the proteinaceous materials to attack by micro-organisms.

The permanent bonding of the fungicidal agent to the fiber and a high degree of water resistance is imparted to the fibrous materials by reason of the resin which may be selected from various urea-formaldehyde and melamine resins. The same resin-forming composition may be used in both the impregnation step and in the second protective step wherein additional water repellency is imparted to the impregnated felt. These resins must be used in the treating solutions in the form of water soluble or water dispersible resin-forming compositions. For the purpose of this invention, I prefer to use a resin-forming composition of the type illustrated by the alkyl ethers of an alkylol

melamine such as the methyl ether of methylol melamine, the methyl ether of dimethylol melamine or the dibutyl ether of tetramethylol melamine. However, other amine - aldehyde resin-forming compositions may be used in either step such as those containing urea-formaldehyde, melamine-formaldehyde, dimethylol urea, or dimethylol urea ethers of lower saturated aliphatic alcohols of one to six carbon atoms. An acidic catalyst is used in conjunction with the resin-forming composition to effect the proper condensation and formation of the resin. While I prefer to use cyclohexyl ammonium phosphate as the catalyst, di-ammonium phosphate, phosphoric acid, acetic acid or formic acid may be substituted. However, in the second treating step, wherein the solution is maintained at a pH of 9 to 10 by the use of a fugitive base, the catalyst should be selected from cyclohexyl ammonium phosphate and di-ammonium phosphate. On the other hand, the copending application No. 551,077 and now Patent No. 2,537,677 discloses that the usual acidic condensation catalyst may be omitted where a N,N'-diacyl diamino methane is used in the second step of the process. In the presence of a N,N'-diacyl diamino methane, the amine-aldehyde condensation will proceed in a neutral solution. But, in this process a catalyst such as the above described ammonium salts may be used if desired. The amount of catalyst is generally about 3 to 4% of the weight of the melamine or urea-formaldehyde resin used.

The impregnation with the fungicidal or bactericidal agent may be accomplished in any desired manner, for example, by immersion of the felt in a vessel containing the treating solution which may be at room temperature and, the impregnation may be handled either as a continuous operation or as a batch process. For the treatment of papermakers' felt I have obtained excellent results by using a padder, mangle or rolls with an adjusted "nip" so as to give the desired "pick-up" of the fungicidal composition. In most instances, a "pick-up" of the fungicidal agent equivalent to 1/2% to 2% of the weight of the untreated felt is most desirable. Likewise, the drying operation may be accomplished in any desired manner, for example, by exposing the respectively treated surfaces simultaneously or successively to air streams which may be at room temperature or at some elevated temperature below the charring point of the fibrous material, preferably about 215° F. With regard to curing, variations with reference to the time and temperature of the cure depend entirely upon the heat setting properties of the resin selected. For example: When I use a melamine type resin-forming composition, the following table indicates the temperature curing time and for the resin after all of the water has been removed from the felt:

|    | Time (minutes) | Temperature °F. |
|----|----------------|-----------------|
| 20 |                | 250             |
| 10 |                | 260             |
| 5  |                | 280             |
| 3  |                | 310             |
| 2  |                | 320             |
| 70 |                |                 |

Likewise, the water soluble urea-formaldehyde resin-forming composition may be cured in 3 to 20 minutes at a temperature of 250 to 300° F.

In the second step of this process, high perma-

hent water repellency is imparted to the impregnated felt. The N,N' diacyl diamino methane may be prepared in the manner described in U. S. Patent No. 2,365,813. Since both the N,N' diacyl diamino methane and the resins which have been hereinbefore described, are water insoluble the application to the textile fiber is most conveniently made by means of an aqueous suspension or dispersion of the diamide, the resin-forming composition and a dispersing agent comprising the fatty acid salt of a fugitive base. The fatty acid used to form the dispersing agent may be any fatty acid saturated, unsaturated or hydroxylated and should have a carbon chain length of at least 12 to 28 carbon atoms. Accordingly, there may be employed lauric, stearic, palmitic or oleic acids or other fatty acids contained within the above length of carbon chain lengths. The fatty acid salt is preferably the ammonium salt although other bases capable of volatilizing at the temperature at which the heat treatment is carried out may also be used. Examples of such bases are morpholine, pyridine, cyclohexlamine and 2-amino-2-methyl-1-propanol. The dispersion contains in addition sufficient ammonia or other fugitive base to bring the hydrogen ion concentration of the dispersion over to the alkaline side of neutrality and preferably to the point where the pH thereof will be within the range of from 9.0 to 10.0. Within this pH range the dispersed diacyl diamino methane and amine-aldehyde resin-forming compositions when reduced by suitable means to a particle size of from 0.5 to 10.0 microns is a stable emulsion both at room temperature and at temperatures as high as 80° C.

Application of the dispersion to the fabric may be made directly by immersion as by treatment in a jig or padder or alternatively by spraying the dispersion upon the textile fabric. While the treatment of the fiber is most conveniently carried out by means of a single dispersion containing both the diacyl diamino methane, the resin-forming composition and the dispersing agent the application may be made by successive treatments of the fabric with a separate dispersion of the diamide and dispersing agent and later with the resin-forming composition.

The amount of "pick-up" of materials from the second immersion depends upon the particular use to which the felt is to be put. However, solids from this immersion may be incorporated into the felt equivalent to 20% to 125% of the weight of the untreated felt.

The application of the aqueous dispersion to the textile product may take place at any temperature between room temperature and up to temperatures as high as 175° F. The treated felt is again dried either at room temperature or in heating air, briefly at about 215° F. After the moisture has been evaporated from the felt the temperature is raised to between 250° F. and 320° F. for 2 to 20 minutes.

#### EXAMPLE I

A water dispersible paste concentrate is first prepared containing:

2.00 parts of copper 8-quinolinolate  
20.00 parts of 5% aqueous solution of methyl celulose  
0.05 part of decyl benzene sodium sulfonate

22.05 parts of the above paste concentrate is dispersed in 75.35 parts of water, to which is added 2.00 parts of a water soluble resin-forming com-

position of an ether of dimethylol melamine containing 0.60 part of a 10% aqueous solution of cyclohexyl ammonium phosphate.

The papermakers' felt is then treated with the prepared fungi proofing composition at room temperature using a mangle. After drying, at 215° F., the treated felt is cured for 3 minutes at a temperature of 300° F.

A second dispersion is prepared containing:

|                                                                                              | Per cent |
|----------------------------------------------------------------------------------------------|----------|
| N,N' distearoyl diamino methane                                                              | 5.0      |
| Solution of a resin-forming composition of dibutyl ether of tetra methylol melamine (solids) | 10.5     |
| 15 Stearic acid                                                                              | 3.5      |
| Ammonium hydroxide 28%                                                                       | 4.0      |
| Cyclohexyl ammonium phosphate                                                                | 0.4      |
| Water                                                                                        | Balance  |

The dispersion is prepared by adding the melted fatty acid to the water, adding the ammonia until a pH of 9.0 to 10 is reached. Finely divided N,N' distearoyl diamino methane (particle size below 10 microns) is added and the mixture passed through a colloid mill. The resin-forming melamine composition added and the whole mixture again passed through the colloid mill. The felt is immersed in the dispersion, at a temperature between room temperature and 100° F., the amount of pick-up being controlled by the nip of the padder rolls. The melt is then dried at 215° F. and finally heat cured at 300° F. for 5 minutes.

The felt, treated as described above, was leached for 1,000 hours with running tap water, and the permanence of the fungi and bacteria proofing treatment is illustrated by the following table:

Table I.—Retentivity of copper 8-quinolinolate in papermakers' felts

|     | Hours Leached With Running Tap Water | Per cent of Copper 8-Quinolinolate in the Felt on a Weight Basis |
|-----|--------------------------------------|------------------------------------------------------------------|
| 45  |                                      |                                                                  |
| 0   |                                      | 1.25                                                             |
| 48  |                                      | 1.21                                                             |
| 100 |                                      | 1.21                                                             |
| 200 |                                      | 1.20                                                             |
| 500 |                                      | 1.20                                                             |
| 50  | 1,000                                | 1.20                                                             |

Samples of the felt which were leached 1,000 hours in running tap water were inoculated with each of the following organisms:

55 *Chaetomium globosum*, *Metarrhizium sp.*, *Aspergillus niger* and *Penicillium sp.* and then incubated for customary periods of time.

Results of the biological test are given below in Table II.

Table II.—Fungus resistance of copper 8-quinolinolate treated felt leached 1,000 hours in running water

|    | Organism                   | Fungus Activity on the Sample            |
|----|----------------------------|------------------------------------------|
| 65 | <i>Chaetomium globosum</i> | No growth of the organism on the sample. |
|    | <i>Metarrhizium sp.</i>    | Do.                                      |
|    | <i>Aspergillus niger</i>   | Do.                                      |
| 70 | <i>Penicillium sp.</i>     | Do.                                      |

Further tests on the treated felt established the fact that the treatment as herein described in no way affected or reduced the tensile strength of the warp or filling of the felt.

## 7

The zinc or cadmium salts of 8-hydroxyquinoline were substituted in the above example with substantially the same results.

The proportion of the ingredients may be varied depending upon the amount of preservative and resin desired in the finished felt. However, the normal desirable range which may be used in varying the proportions of the various ingredients in the impregnation treatment are as follows:

|                                                                                                              |    |
|--------------------------------------------------------------------------------------------------------------|----|
| 1.00-3.0% copper, zinc or cadmium 8-quinolinolate, 5,7-dichlor-8-quinolinolate or 5,7-dibrom-8-quinolinolate | 10 |
| 10.00-30.0% 5% aqueous solution methyl cellulose                                                             | 15 |
| 0.05-2.0% wetting agent                                                                                      |    |
| 0.50-20.0% melamine or urea-formaldehyde resin in a resin-forming composition form                           |    |
| 0.15-3.0% 10% aqueous solution of catalyst                                                                   | 20 |
| 88.30-52.0% water                                                                                            |    |

In addition, the normal desirable range which may be used in varying the preparations of the various ingredients in the step wherein the water repellency is insured, is as follows:

|                                               | Per cent |
|-----------------------------------------------|----------|
| N,N' diacyl diamino methane                   | 3.5-15   |
| Melamine or amine-formaldehyde resin (solids) | 8.0-24   |
| Fatty acids                                   | 3.5- 8   |
| Fugitive base                                 | 4.0- 8.0 |
| Condensation catalyst                         | 0.0- 1.0 |
| Water                                         | Balance  |

The dispersion may also be varied somewhat by replacing up to 50% of the N,N' diacyl diamino methane with other well known water repellents as aluminum stearate, a paraffin wax, or N-methylol alkyl amide wherein the alkyl chain has 12 to 28 carbon atoms.

## EXAMPLE II

## Water dispersible paste concentrate

|                                                  |  |
|--------------------------------------------------|--|
| 3.00 parts of copper 5,7-dichlor-8-quinolinolate |  |
| 0.75 parts of decyl benzene sodium succinate     |  |
| 30.00 parts of carboxy methyl cellulose          |  |

## Ready to use treating solution

|                                                                           |  |
|---------------------------------------------------------------------------|--|
| 33.75 parts of the above paste concentrate                                |  |
| 4.00 parts of a water soluble urea-formaldehyde resin-forming composition |  |
| 0.16 part of phosphoric acid                                              |  |
| 62.19 parts of water                                                      |  |

The felt is run through the treating solution at room temperature, oven dried at 215° F. and finally cured by heating for 10 minutes at 275° F.

The treating solution for imparting increased water repellency to the felt may be prepared as follows:

|                                                      | Per cent |
|------------------------------------------------------|----------|
| N,N' distearoyl diamino methane                      | 3.5      |
| N methylol stearamide                                | 3.5      |
| Urea-formaldehyde resin-forming composition (solids) | 15.0     |
| Oleic acid                                           | 3.5      |
| Triethanol amine                                     | 4.0      |
| Cyclohexyl ammonium phosphate                        | 0.6      |
| Water                                                | Balance  |

The dispersion is made as described in Example I. The felt is run through the treating solution at 100° F., dried at 215° F. and again cured by heating for 10 minutes at 275° F.

The 1,000-hour leaching test gave substantially the same results as in Example I, and inoculation of the leached samples with *Chaetomium*

## 8

*globosum*, *Metarrhizium* sp., *Aspergillus niger* and *Penicillium* sp. and incubation produced no growth of any organism on the samples.

The zinc and cadmium salts of 5,7-dibrom-8-quinolinolate indicated substantially the same results, that is, high and permanent resistance to fungal and bacterial activity.

## EXAMPLE III

## Water dispersible paste concentrate

|                                                           |  |
|-----------------------------------------------------------|--|
| 1.00 part of copper 5,7-dibrom-8-quinolinolate            |  |
| 0.05 part of a poly-glycol ether of di-isobutylene phenol |  |
| 10.00 parts of casein                                     |  |

## Ready to use treating solution

|                                                          |  |
|----------------------------------------------------------|--|
| 11.05 parts of above paste concentrate                   |  |
| 5.00 parts of a water soluble ether of methylol melamine |  |
| 0.15 part of diammonium phosphate                        |  |
| 83.80 parts of water                                     |  |

The felt is run through the treating solution at room temperature, oven dried at 215° F. and finally cured by heating for 3 minutes at 300° F.

A satisfactory emulsion for the second step of the process comprises the following:

|                                                                                    | Per cent |
|------------------------------------------------------------------------------------|----------|
| N,N' distearoyl diamino methane                                                    | 2.0      |
| Aluminum stearate                                                                  | 2.0      |
| Water soluble resin-forming composition of the methyl ether of dimethylol melamine | 8.0      |
| Lauric acid                                                                        | 5.0      |
| 2-amino-2-methyl-1-propanol                                                        | 5.0      |
| Diammonium phosphate                                                               | 0.3      |
| Water                                                                              | Balance  |

The dispersion is prepared in the manner described in Example I, and the felt run through the dispersion until a weight of solids equivalent to about 40% of the weight of the dry untreated felt is picked up. The felt is dried at 215° F. and finally heat cured for 5 minutes at 280° F.

The 1,000-hour leaching test gave substantially the same results as in Example I, and inoculation of the leached samples with *Chaetomium globosum*, *Metarrhizium* sp., *Aspergillus niger* and *Penicillium* sp., and incubation produced no growth of any organism on the samples.

The zinc and cadmium salts of 5,7-dibrom-8-quinolinolate indicated substantially the same results, that is, high and permanent resistance to fungal and bacterial activity.

I claim:

1. A process for increasing the resistance of fibrous materials to the activity of fungi and bacteria comprising contacting the fibrous material with an aqueous composition containing a relatively water insoluble 8-quinolinolate selected from the group consisting of copper, zinc and cadmium derivatives of 8-quinolinol, 5,7-dibrom-8-quinolinol and 5,7-dichlor-8-quinolinol, a film-forming protective colloid, a surface active agent, a resin-forming amine-aldehyde composition, and an amine-aldehyde condensation catalyst; drying the impregnated fibrous material; heating the impregnated fibrous material for 3 to 20 minutes at 250 to 320° F.; contacting the impregnated fibrous material with an aqueous composition containing a water repellent, a resin-forming amine-aldehyde composition, an amine-aldehyde condensation catalyst and a dispersing agent comprising a fatty acid salt of a fugitive base; drying the impregnated fibrous material, and heating the impregnated fibrous material for 3 to 20 minutes at 250-320° F.

2. A process for increasing the resistance of fibrous materials to the activity of fungi and bacteria comprising contacting the fibrous material with an aqueous composition containing 1-3% of a relatively water insoluble 8-quinolinolate selected from the group consisting of the copper, zinc and cadmium derivatives of 8-quinolinol, 5,7-dibrom-8-quinolinol and 5,7-dichlor-8-quinolinol, 0.5-2% of a film-forming protective colloid, 0.5-20% of an amine-aldehyde resin-forming composition, 0.1-3% of an amine-aldehyde condensation catalyst, and 0.05-2% of surface active agent; drying the impregnated fibrous material; heat curing the impregnated fibrous material for 3 to 20 minutes at 250-320° F.; contacting the heat cured impregnated fibrous material with an aqueous composition containing 3-15% of a diacyl diamino methane wherein the acyl group is derived from a fatty acid having 12 to 28 carbon atoms, 5-25% of an amine-aldehyde resin-forming composition, 0.1-3% of an amine-aldehyde condensation catalyst, 3.5-8% of a dispersing agent; drying the impregnated fibrous material and heat curing the impregnated fibrous material for 3-20 minutes at 250-320° F.

3. A process for increasing the resistance of fibrous materials to the activity of fungi and bacteria comprising contacting the fibrous material with an aqueous composition containing 1-3% of a relatively water insoluble 8-quinolinolate selected from the group consisting of the copper, zinc and cadmium derivatives of 8-quinolinol, 5,7-dibrom-8-quinolinol and 5,7-dichlor-8-quinolinol, 0.5-2% of a film-forming protective colloid, 0.5-20% of a resin-forming melamine ether, and 0.1-3.0% of a melamine condensation catalyst; drying the impregnated fibrous material; heat curing the impregnated fibrous material for 3 to 20 minutes at 250-320° F.; contacting the heat cured impregnated fibrous material with an aqueous composition containing 3-15% of a diacyl diamino methane wherein the acyl group is derived from a fatty acid having 12 to 28 carbon atoms, 0.5-20% of a resin-forming melamine ether, 0.1-3.0% of a melamine condensation catalyst, 3.5-8% of a fatty acid, and 4-8% of a fugitive base; drying the impregnated fibrous material and heat curing the impregnated fibrous material for 3-20 minutes at 250-320° F.

4. Process of claim 3 wherein the resin-forming melamine ether is the tetra butyl ether of tetra methylol melamine.

5. A process for increasing the resistance of fibrous materials to the activity of fungi and bacteria comprising contacting the fibrous material with an aqueous composition containing 1-3% of a relatively water insoluble 8-quinolinolate selected from the group consisting of copper, zinc and cadmium derivatives of 8-quinolinol, 5,7-dibrom-8-quinolinol and 5,7-dichlor-8-quinolinol, 0.5-2% of a film-forming protective colloid, 0.5-20% of the resin-forming dibutyl ether of tetra methylol melamine, and 0.1-3.0% of a melamine ether condensation catalyst; drying the impregnated fibrous material; heat curing the impregnated fibrous material for 3 to 20 minutes at 250-320° F.; contacting the heat cured impregnated fibrous material with an aqueous composition containing 3-15% of N,N' distearoyl diamino methane, 0.5-20% of the resin-forming dibutyl ether of tetra methylol melamine, 0.1-3.0% of a melamine ether condensation catalyst, 3.5-8% of a fatty acid, and 4-8% of a fugitive base; drying the impregnated fibrous material and heat

curing the impregnated fibrous material for 3-20 minutes at 250-320° F.

6. A process for increasing the resistance of papermakers' felts to the activity of fungi and bacteria comprising contacting the felt with an aqueous composition containing 1-3% of a relatively water insoluble 8-quinolinolate selected from the group consisting of copper, zinc and cadmium derivatives of 8-quinolinol, 5,7-dibrom-8-quinolinol and 5,7-dichlor-8-quinolinol, 0.5-2% of a film-forming protective colloid, 0.05-2% of a surface active agent, 0.5-20% of a resin-forming melamine ether, and 0.1-3.0% of a melamine ether condensation catalyst; drying the impregnated felt; heat curing the impregnated felt for 3 to 20 minutes at 250 to 320° F.; contacting the heat cured impregnated felt with an aqueous composition containing 3 to 15% of a diacyl diamino methane wherein the acyl group is derived from a fatty acid having 12 to 28 carbon atoms, 5 to 25% of a resin-forming melamine ether, 3 to 8% of a fatty acid salt of a fugitive base; drying the impregnated felt, and heat curing the impregnated felt for 3 to 20 minutes at 250 to 320° F.

7. A process for increasing the resistance of papermakers' felts to the activity of fungi and bacteria comprising dispersing a paste concentrate comprising two parts of copper-8-quinolinolate, 20 parts of 5% aqueous solution of methyl cellulose and 0.05 part of a wetting agent with an aqueous resin-forming composition containing 75 parts of water, 2 parts of the dibutyl ether of tetra methylol melamine and 0.6 part of 10% aqueous solution of cyclohexyl ammonium phosphate; contacting the felt with the above described water dispersion; drying the impregnated felt; heat curing the impregnated felt for 3 to 20 minutes at 250-320° F.; contacting the cured impregnated felt with an aqueous dispersion containing 5% N,N' distearoyl diamino methane, 10% of a resin-forming dibutyl ether of tetra methylol melamine; 3.5% of stearic acid, 4% of 28% ammonium hydroxide and 72.5% water; drying the treated felt and heat curing for 3 to 20 minutes at 250-320° F.

8. A water repellent papermakers' felt possessing increased resistance to the activity of fungi and bacteria comprising a papermakers' felt containing within its interstices a relatively water insoluble 8-quinolinolate selected from the group consisting of the copper, cadmium and zinc derivatives of 8-quinolinol, 5,7-dibrom-8-quinolinol and 5,7-dichlor-8-quinolinol, a water repellent, and a resinous amine-aldehyde condensation product; said felt having been impregnated with an aqueous dispersion containing the 8-quinolinolate, a protective colloid, a wetting agent, a resin-forming amine-aldehyde composition and an amine-aldehyde condensation catalyst, dried and heated to effect the condensation of the amine-aldehyde composition to form the resinous amine-aldehyde condensation product, and having been subsequently treated with an aqueous dispersion containing the water repellent, a dispersing agent, and the resin-forming amine-aldehyde composition; dried and heated to effect the condensation of the amine-aldehyde composition to form the resinous condensation product.

9. A water repellent papermakers' felt possessing increased resistance to the activity of fungi and bacteria comprising a papermakers' felt containing within its interstices a relatively water insoluble 8-quinolinolate selected from the group consisting of the copper, cadmium and zinc derivatives of 8-quinolinol, 5,7-dibrom-8-quinolinol

## 11

and 5,7-dichlor-8-quinolinol, a N,N' diacyl di-  
amino methane wherein the acyl group is derived  
from fatty acids of 12 to 28 carbon atoms, and a  
resinous melamine ether condensation product;  
said felt having been impregnated with an aque-  
ous dispersion containing the 8-quinolinolate, a  
protective colloid, a wetting agent, a resin-form-  
ing melamine ether and a melamine ether con-  
densation catalyst, dried and heated to effect the  
condensation of the melamine ether to form the  
resinous melamine condensation product, and hav-  
ing been subsequently treated with an aqueous  
dispersion containing the N,N' diacyl diamino  
methane, a dispersing agent, and the resin-form-  
ing melamine ether, dried and heated to effect the  
condensation of the melamine ether to form the  
resinous condensation product.

10. A water repellent papermakers' felt possess-  
ing increased resistance to the activity of fungi  
and bacteria comprising a papermakers' felt con-  
taining within its interstices copper-8-quinolino-  
late, N,N' distearoyl diamino methane and a res-  
inous condensation product of the dibutyl ether  
of tetra methylol melamine; said felt having been  
impregnated with an aqueous dispersion contain-  
ing the copper-8-quinolinolate, a protective col-

loid, a wetting agent, a resin-forming dibutyl  
ether of tetra methylol melamine, and a melamine  
ether condensation catalyst; dried and heat cured  
to effect the condensation of the melamine ether  
5 to form the resinous melamine condensation prod-  
uct, and subsequently treated with an aqueous dis-  
persion containing the N,N' distearoyl diamino  
methane, a dispersing agent comprising a fatty  
acid salt of a fugitive base, and a resin-forming  
10 dibutyl ether of tetra methylol melamine, dried  
and heated to form the resinous melamine con-  
densation product.

## 12

PAUL GEORGE BENIGNUS.

## REFERENCES CITED

The following references are of record in the  
file of this patent:

## UNITED STATES PATENTS

| Number    | Name           | Date          |
|-----------|----------------|---------------|
| 2,111,698 | Siefert et al. | Mar. 22, 1938 |
| 2,191,362 | Widmer et al.  | Feb. 20, 1940 |
| 2,282,988 | Creely         | May 12, 1942  |
| 2,381,863 | Benignus       | Aug. 14, 1945 |
| 2,423,185 | Gundel et al.  | July 1, 1947  |